

Patented Nov. 8, 1932

1,886,441

# UNITED STATES PATENT OFFICE

JAMES STEVENSON WILSON AND JOHN THOMAS, OF GRANGEMOUTH, SCOTLAND,  
ASSIGNORS TO SCOTTISH DYES, LIMITED, OF GRANGEMOUTH, SCOTLAND

## DYEING CELLULOSE ACETATE

No Drawing. Application filed November 21, 1929, Serial No. 408,921, and in Great Britain  
November 27, 1928.

This invention relates to the dyeing of cellulose acetate with ester salts of vat dyestuffs.

The object of the present invention is to provide an improved or modified process for 5 the dyeing of cellulose acetate with ester salts of vat dyestuffs.

As a result of researches, we have found that acetyl silk can be dyed by the same method as cotton or wool, without the necessity 10 for prolonged steaming, or for in fact, in many cases, the application of any steaming process, although it may sometimes be necessary to scour the acetyl silk before dyeing, to remove gum or size used in weaving or other 15 processes.

The invention in brief consists in the application to the dyeing of cellulose acetate or acetyl silk with ester salts of vat dyestuffs 20 of processes as used for the dyeing of cotton or wool or silk with such bodies, scouring of the acetate when in the form of acetyl silk or the like before dyeing being practised, when necessary to remove gum or size introduced 25 in connection with weaving or other processes.

The invention also consists in a method of dyeing cellulose acetate or acetyl silk which comprises the following steps:—

30 Heating the bath,  
Treatment of the acetyl silk,  
Introduction of salt, and

35 Further treatment of the acetyl silk,  
the shade subsequently being developed.

The invention also consists in a method of dyeing cellulose acetate or acetyl silk which consists in a prolonged dyeing treatment.

40 The invention also consists in methods for dyeing cellulose acetate or acetyl silk substantially as herein described, and in products which may be obtained by these methods.

The following examples illustrate how the 45 invention may be carried into effect, references to parts being to parts by weight.

### Example 1

This is an example of the dyeing of cellulose acetate silk with Soledon jade green corresponding to Caledon jade green. Colour 50 Index No. 1101.

For 10 parts of material, 1 part of soledon jade green is dissolved in 400 parts of water. The bath is heated to 50° C., and the previously scoured and wetted-out acetyl silk is then entered. The material is worked for fifteen 55 minutes at this temperature, and then 100 per cent. of salt, calculated on the weight of the acetyl silk material, is added. Dyeing is continued for one hour, and the material is then lifted, squeezed and developed by immersion 60 in a bath containing 1 per cent. of sodium nitrite and 1 per cent. of hydrochloric acid. Development takes place immediately, at normal temperatures, and the goods are rinsed, 65 soaped and dried. A bright green shade is obtained which is fast to washing.

### Example 2

This is another example using Soledon 70 jade green.

The bath is made up in the same way as in Example 1, but with the dye-bath only half the previous volume. The dye-bath is heated to 80° C., the material entered and kept at 75 this temperature for an hour, when it is removed and developed. Development may be carried out at 60° C. in a bath containing 1 per cent. of ferric chloride and 1 per cent. hydrochloric acid. The product is then 80 rinsed, washed and soaped. A bright fast green shade is obtained.

### Example 3

Soledon brilliant purple RR corresponding to Caledon brilliant purple RR. Colour 85 Index No. 1104 is used in this example.

For 10 parts of acetyl silk, the bath is made up by dissolving 1 part of Soledon brilliant purple RR in 400 parts of water with the ad- 90

dition of one-eighth part of dispersol. The dye-bath is heated to 60° C., and the material entered. After fifteen minutes dyeing, 100 per cent. of salt, calculated on the weight of the silk, is added, and dyeing continued for another hour. The material is then removed

### Example 6

This example illustrates the various dye-stuffs which may be used, and the resulting shades obtained on different kinds of acetyl silk:—

|                                                                            | Method A.                       | Method B.                        | Method C.                        | 75 |
|----------------------------------------------------------------------------|---------------------------------|----------------------------------|----------------------------------|----|
|                                                                            |                                 |                                  |                                  |    |
| 10                                                                         | 10 per cent on celanese tricot. | 10 per cent on acetyl silk yarn. | 3 per cent on acetyl silk cloth. | 75 |
| Indigosol yellow HGG                                                       | Pale gold-orange                | Pale gold-orange                 | Golden yellow tint.              |    |
| Indigosol golden yellow IGK                                                | Strong bright yellow            | Strong bright yellow             | Medium bright yellow.            |    |
| Indigosol red HR                                                           | Deep bright pink                | Deep bright pink                 | Pale pink.                       |    |
| Indigosol violet AZB                                                       | Bright violet                   | Bright violet                    | Lilac shade.                     |    |
| Indigosol green AB                                                         | Deep bright green               | Deep bright green                | Pale apple green.                |    |
| Indigosol orange HR                                                        | Medium apricot                  | Medium apricot tint.             | Pale apricot.                    | 80 |
| Indigosol red HCR                                                          | Medium brownish-red             | Medium brownish-red              | Pale pink.                       |    |
| Indigosol scarlet HB                                                       | Bright pink                     | Bright pink                      | Pale pink.                       |    |
| Indigosol HB                                                               | Deep reddish-blue               | Deep bright violet               | Pale violet.                     |    |
| Indigosol OR                                                               | Medium blue                     | Bright greyish-blue              | Pale grey-blue.                  |    |
| Indigosol AZG                                                              | Greenish-blue                   | Greenish-blue                    | Pale greenish-blue.              |    |
| Indigosol O4B                                                              | Bright blue                     | Deep bright blue                 | Pale blue.                       |    |
| Indigosol black IB                                                         | Greyish-black                   | Greyish-black                    | Pale greenish-grey.              |    |
| Indigosol blue O                                                           | Pale grey-blue                  | Medium bluish-grey               | Grey tint.                       | 85 |
| Indigosol pink HR                                                          | Bright pink                     | Bright pink                      | Pale pink.                       |    |
| Indigosol red violet IRH                                                   | Bright red-violet               | Bright red-violet                | Pale purple.                     |    |
| Indigosol O6B                                                              | Greenish-blue                   | Deep bright blue                 | Pale green.                      |    |
| Soledon jade green                                                         | Deep bright green               | Deep bright green                | Pale green.                      |    |
| Soledon yellow G corresponding to Caledon yellow G. Colour Index No. 1118. | Pale dull yellow                | Medium dull yellow               | Cream.                           |    |
| Soledon purple R corresponding to Caledon purple R. Colour Index No. 1103. | Deep bright purple              | Deep bright purple               | Pale purple.                     | 90 |

and developed. Development may be done as follows:—The goods are passed first through a cold solution of 1 per cent. sodium nitrite, and then through a cold solution of 1 per cent. hydrochloric acid, rinsed and soaped.

### Example 4

35 This is an example of the use of Indigosol O4B.

The dye-bath is made up in a similar manner to Example 1 and dyeing carried out at 40 60° C. with the use of salt, except that the material is only immersed for half an hour after the addition of the salt. Development may be carried out in a bath containing 1 per cent. of potassium persulphate and 1 per cent. 45 of sulphuric acid at 70° C.

### Example 5.

Indigosol golden yellow IGK is used in this 50 example.

For 10 parts of acetyl silk cloth the bath is made up by dissolving 0.25 part of Indigosol golden yellow IGK in 200 parts of water containing 4 parts of sodium nitrite.

55 The dye-bath is heated to 75° C., and the melted-out material entered. After fifteen minutes dyeing, 10 parts of salt are added and dyeing continued for forty-five minutes. The material is then removed and developed

60 by immersion in a cold 1 per cent. hydrochloric acid solution. After development the material is rinsed and soaped in a bath containing 1 per cent. soap at 40° C. for fifteen minutes. After soaping, the material is well 65 rinsed and dried.

The above dyeing is obtained by the following method:—

1 part of colour is carefully pasted with 1 part of a sulphonated castor oil. To this is added 5 parts of water. The whole is added to 200 parts of water at 75° C. 10 parts of the material, which has been previously well scoured in 1 per cent. soap, 0.2 per cent. soda and 0.2 per cent. ammonia is entered into this liquor, and dyeing carried on for thirty minutes, while the temperature is carefully raised to 80° C. At the end of this period, 1 part of salt is added, and dyeing carried out for a further ten minutes, when a further 1 part of salt is again added. The dyeing is then completed after a further fifteen minutes. The temperature during the latter period is maintained at 80° C.

105 In the above method the amount of liquor used can be varied from 100 parts to 400 parts according to the dyestuff used.

110 At the end of the dyeing operation the material is lifted, squeezed and developed by immersion in a bath containing 2 per cent. of sodium nitrite and 2 per cent. of sulphuric acid. Development takes place readily at normal temperatures. The material is then lifted, rinsed, soaped in a bath containing 1 per cent. soap at 40° C. for fifteen minutes, rinsed and then dried.

### General

115 The colour index number and other identification of many of the Indigosol dyes listed may be found in the 1928 supplement of the "Society of Dyers and Colourists" but to render this disclosure as complete as possible 120

the following information or index is given—

|                                                                                 |                                                                                                                                       |    |
|---------------------------------------------------------------------------------|---------------------------------------------------------------------------------------------------------------------------------------|----|
| Indigosol yellow HCG.                                                           | Colour Index 1176, see also supplement.                                                                                               |    |
| Indigosol violet AZB.                                                           | According to the supplement to the Colour Index this is the sodium salt of the disulphuric ether of leuco alizarine indigo-violet BZ. |    |
| 5 Indigosol orange HR.                                                          | Colour Index No. 1217. See also supplement.                                                                                           | 70 |
| Indigosol red HCR.                                                              | According to the Colour Index supplement this is the sodium salt of the disulphuric ether of leuco helindone red CR.                  |    |
| 10 Indigosol scarlet HB.                                                        | According to the Colour Index supplement, this is the sodium salt of the disulphuric ether of leuco helindone scarlet B.              | 75 |
| Indigosol HB.                                                                   | According to the Colour Index supplement this is derived from helindone blue B.                                                       |    |
| Indigosol OR.                                                                   | Colour Index No. 1182, see also supplement.                                                                                           |    |
| 15 Indigosol AZG.                                                               | Colour Index No. 1202, see also supplement.                                                                                           | 80 |
| Indigosol O4B.                                                                  | Colour Index No. 1184, see also supplement.                                                                                           |    |
| Indigosol black IB.                                                             | According to the Colour Index supplement, this is the sodium salt of the disulphuric ether of leuco thioindigo black B.               |    |
| 20 Soledon jade green corresponds to Caledon jade green, Colour Index No. 1101. |                                                                                                                                       | 85 |

It is sometimes necessary to scour the acetyl silk before dyeing to remove gum or size used in weaving or other processes. The method is applicable not only to acetyl silk itself, but also to acetyl silk in admixture with other materials. In such mixtures either solid shades or shades in which one material is dyed more deeply than the other can be obtained, the results depending on the conditions used.

In dyeing the union material containing natural silk and acetyl silk, greater depth may be obtained on the natural silk if the dyeing is carried out for a short period only.

35 In this specification and claims the term "vat dyestuff enolic ethereal salt" means a soluble salt of a vat dyestuff containing one or more acidic groups attached to the oxygen atoms of the ketonic groups.

40 Having now described our invention, what we claim as new and desire to secure by Letters Patent is:—

1. A process for dyeing cellulose acetate which consists in impregnating the aforesaid cellulose acetate with a vat dyestuff enolic ethereal salt by heating in an aqueous solution and developing the vat dyestuff.

45 2. A process for the dyeing of cellulose acetate, which consists in immersing the cellulose acetate in a previously heated bath of a vat dyestuff enolic ethereal salt at a temperature between about 50° C. and about 80° C., and developing the vat dyestuff.

55 3. A process for the dyeing of cellulose acetate which consists in immersing the cellulose acetate in a previously heated bath of a vat dyestuff enolic ethereal salt, at a temperature of between about 50° C. and about 80° C., maintaining this temperature for about half an hour to about one hour, and developing the vat dyestuff.

60 4. A process for the dyeing of cellulose acetate with vat dyestuff enolic ethereal salts which consists in suspending cellulose acetate

in a previously heated aqueous saline solution of a vat dyestuff enolic ethereal salt, which saline solution contains a salt chosen from the group consisting of sodium sulphate and sodium chloride at a temperature of from about 50° C. to about 80° C. for from about half an hour to about the hour, and developing the vat dyestuff.

5. A process for the dyeing of cellulose acetate in the form of acetyl silk with vat dyestuff enolic ethereal salts which consists in scouring the acetyl silk, suspending the thus scoured acetyl silk in a previously heated aqueous saline solution of a vat dyestuff enolic ethereal salt, which saline solution contains a salt chosen from the group consisting of sodium sulphate and sodium chloride, at a temperature of between about 50° C. and about 80° C. for about half an hour to about one hour, and developing the vat dyestuff.

6. A process for dyeing cellulose acetate, which consists in immersing the cellulose acetate in a previously heated bath of a vat dyestuff enolic ethereal salt, and developing the vat dyestuff in the presence of a salt chosen from the group consisting of sodium sulphate and sodium chloride.

7. A process for the dyeing of cellulose acetate which consists in immersing the cellulose acetate in a previously heated bath of a vat dyestuff enolic ethereal salt, at a temperature of between about 50° C. and about 80° C., maintaining this temperature for about half an hour to about one hour, adding a salt chosen from the group consisting of sodium sulphate and sodium chloride during this stage and developing the vat dyestuff.

8. A process for the dyeing of cellulose acetate in the form of acetyl silk with vat dyestuff enolic ethereal salts which consists in scouring the acetyl silk, suspending the thus scoured acetyl silk in a previously heated aqueous solution of a vat dyestuff enolic ethereal salt at a temperature of between about 50° C. and about 80° C. for about half an hour to about one hour, adding a salt chosen from the group consisting of sodium sulphate and sodium chloride during this stage and developing the vat dyestuff.

In testimony whereof we have signed our names to this specification.

JAS. S. WILSON.  
J. THOMAS.